

3,795,505

PRODUCTION OF DEOXIDATED, DEPURATED,  
KILLED AND REFINED STEELS USING  
ALUMINUM-LITHIUM ALLOYS

Dante Corradini, Via Cacciolepori 11, Milan, Italy  
No Drawing, Continuation-in-part of application Ser. No. 145,049, May 19, 1971, which is a continuation of application Ser. No. 633,714, Apr. 26, 1967, both now abandoned. This application Oct. 18, 1971, Ser. No. 190,402

Claims priority, application Italy, Apr. 7, 1967,  
14,703/67

Int. Cl. C21c 7/08

U.S. Cl. 75—53

1 Claim

## ABSTRACT OF THE DISCLOSURE

The invention relates to the use of alloys consisting essentially of aluminum-lithium for the purpose of deoxidizing, depurating, killing and refining any kind of carbon- or alloy-steel.

The alloys used in the process of the invention contain from 50 to 99.7% of aluminum and from 0.3 to 8% of lithium; they may also suitably contain at least one element selected from the group consisting of rare earths (TR), Ca, Ba, Fe and B, in percentage ranges as follows: Fe 0.5-20%; TR 0.5-13%; Ca 0.2-8%; Ba 0.2-2%.

This application is a continuation-in-part of copending application Ser. No. 145,049 filed May 19, 1971, now abandoned, which in turn is a streamlined continuation of application Ser. No. 633,714 filed Apr. 26, 1967, now abandoned.

The present invention relates to alloys consisting of or comprising aluminium-lithium for the purpose of deoxidizing, depurating, killing and refining low, high and medium carbon steels, and also alloy-steels. The invention provides also the method for the production of such steels deoxidated, depurated, killed and refined by the above mentioned alloys, which greatly improve their physical-mechanical characteristics.

More particularly the present invention relates to aluminium-alloys which comprise from 50 to 99.7% of aluminium and from 0.3 to 8% of lithium. All percentage referred in the present application are by weight.

As it is well known, the most detrimental non-metallic impurities contained in the steels, at the elementary or combined state, are: oxygen, hydrogen, nitrogen and sulphur.

For a long time aluminium has been employed to deoxidate, kill and refine steels, but it produces alumina inclusions and forms aluminium nitride which may impart poor engineering properties to the steel. Moreover the aluminium seems to influence the distribution and the type of the metal sulfide inclusions and, depending on the quantity of aluminium added to the liquid steel, the sulfide inclusions may assume such distributions which are highly harmful to the characteristics of the steels.

Aluminum alloys, containing from 0 up to 95% of various metals including lithium, for depurating steel were proposed in an English patent of 1902.

Later on in 1927, in an American patent relating to structural Al-Li alloys it is affirmed that similar alloys, proposed for depurating steel, are unsuitable for structural alloys, because they contain more than 40% of lithium.

Notwithstanding these antecedents, or perhaps owing to these antecedents Li-Al alloys were afterwards no more considered for depurating molten steel, as can be drawn e.g. from the Revue de Metallurgie, 1963, where methods for adding metal lithium to molten steel are considered and where it is concluded that such methods—often asso-

ciated with argon bubbling through the molten steel—are unsatisfactory because of explosion danger and because only a small percentage of the added lithium is utilized while the greatest part is lost through evaporation; the boiling point of Li being of 1325° C.

However, it was confirmed that lithium additions to molten steel can notably improve its mechanical characteristics, in that it lowers the oxygen, nitrogen, hydrogen and sulphur content of the steel, it allows a reduction of inclusions and exerts a grain refining action.

On the other hand it was within the prior art knowledge that lithium reacts with the moisture in the air, which reaction of course must be avoided in order not to introduce hydrogen and oxygen in the steel with the lithium addition.

It was also known that liquid lithium will react with virtually every other material including refractories and that lithium oxide has a quite remarkable solvent action on almost all known refractory materials, which may therefore pollute the steel.

There are also known for the treatment of steel, aluminium-rare earths alloys (the term "rare earths," TR, issued to mean a mixture of metals of the lanthanides group, commercially named "Mischmetal" which contains approximately: cerium 46-52%, lanthanum 24-27%, neodyum 14-18% the remaining material being constituted by other elements of the rare earth group).

However, although these alloys represent a certain progress when compared with the use of pure aluminium, they do not solve the inclusions problem as the rare earths do in no way react with the formed  $Al_2O_3$  in order to eliminate it; moreover the rare earth oxides and sulfides formed by reaction with oxygen and sulphur, remain in the steel.

This being the situation of the prior art I endeavoured to find a way of introducing lithium in molten steel avoiding the inconveniences above reported.

In so far as the binary alloys Al-Li are concerned, I have found that if the content of Li is of about 0.3% or less, the alloy will practically act as if composed by pure Al.

I have also found that Al-Li alloys are stable in usual storage conditions, that is in contact with the atmosphere, only if the Li content is lower than 1.2%.

Further I have found that it is possible to prepare Al-Li Alloys, stable to storage and with a Li content higher than 1.2% by addition to the Al-Li alloy of at least one of the following elements in the indicated percentages

|    | Percent |
|----|---------|
| Ca | 0.2-8   |
| TR | 0.5-13  |
| Fe | 0.5-20  |
| Ba | 0.2-2   |

Further I have found that also in the thus stabilized alloys, the Li content may not be higher than 8%, otherwise when adding the alloy to the ladle it may cause dangerous molten steel projection, refractories corosions, contamination of the steel by  $Al_2O_3$  inclusions, etc. For example, a Al-Li-Fe alloy having 8% of Li, 10% of Fe and 82% of Al, is a quite stable one.

I have further found that the addition of TR, Ca, Ba, to the Al-Li alloys of the invention, within the given limits, provide the following advantages:

a much better elimination of the impurities  $O_2$ ,  $N_2$ ,  $S$ ,  $H$  and of the  $Al_2O_3$  inclusions and prevention of AlN formation;  
a much better killing and refining action;  
a higher yield of the alloy components;  
a practically total elimination of the refractory etching.

One portion of rare earths added to the new alloys hereabove described correspond, for the purpose of the present invention, approximately 0.5 parts of cerium or to 0.2 parts of lanthanum.

Furthermore I have found that by adding from 0.2 to 1.7% of boron to the ternary alloys Al-Li-TR, it is possible to introduce this element into the steel without boron nitride formation (which causes steel embrittlement) thus achieving, besides the advantages hereabove specified, higher and constant boron yields, much superior to those usually obtained employing the known boron-alloys manufactured for such purpose.

Various other elements may be added to the alloys of the present invention such as: Si, Mn, Ni, Ti, Zr, Fe, Y, Mg. Depending on the element used, either an economic advantage may be obtained or a special steel endowed with peculiar characteristics.

In any case, in order to attain the principal object of the present invention, the alloys must have an Al content higher than 50%, the lithium content being always comprised between 0.3 and 8%. In order to demonstrate that the following percentages of Li: 0.3, 1.2 and 8%, in the Al alloys are critical, experiments A, B, C were carried out. In Example I, II and III the performances of steels treated with the alloys of the invention are reported.

In experiments A, B and C, the amount of alloy added was always kept in the range of 1% by weight of the steel.

#### EXPERIMENTS A

Al-Li alloy containing 0.35% of Li was used with a steel of the following composition: C 0.18%—Mn 0.84%—Si 0.32%—P+S 0.06%.

Microprobe analysis of the steel inclusions, gave the following results: total inclusions 197 p.p.m., FeO 16%; Al<sub>2</sub>O<sub>3</sub> 34%; SiO<sub>2</sub> 36%; MnO 6%; others 8%. By using the same percentage, namely 1%, of pure aluminum, the following results were obtained: total inclusions 195 p.p.m., FeO 15%; Al<sub>2</sub>O<sub>3</sub> 35%; SiO<sub>2</sub> 34%; MnO 7%, others 9%. The amount of inclusions does not practically differ in the two cases.

The reported results each of which represent the weighted mean of five experiments, clearly show that an Al-Li alloy with 0.35% of Li has practically no effect on the steel.

#### EXPERIMENTS B

Al-Li alloys containing 1, 1.2, 1.5% of Li were stored for 1 year. After this storage time the initial color of the alloy with 1.5% of Li had changed from pale grey to dark grey and the surface of this alloy presented a few scales which were removed with a steel brush before using the alloy.

The same steel and technique as in Experiment A were used throughout.

With pure Al: total inclusions 195 p.p.m.; FeO 15%; Al<sub>2</sub>O<sub>3</sub> 35%; SiO<sub>2</sub> 34%; MnO 7%, others 9%.

Alloy Al-Li with 1% Li: total inclusions 107 p.p.m.; FeO 7.4%; Al<sub>2</sub>O<sub>3</sub> 16%; SiO<sub>2</sub> 32%; MnO 22%; others 22.6%.

Alloy Al-Li with 1.2% Li: total inclusions 103 p.p.m.; FeO 9.4%; Al<sub>2</sub>O<sub>3</sub> 15.6%; SiO<sub>2</sub> 30%; MnO 22%; others 23%.

Alloy Al-Li with 1.5% Li: total inclusions 91 p.p.m.; FeO 9%; Al<sub>2</sub>O<sub>3</sub> 15%; SiO<sub>2</sub> 20%; MnO 25%; others 20%.

#### EXPERIMENTS C

The following alloys were used, compositions in percentage,

| Alloy number: | Al | Li | TR | Ca | Fe |
|---------------|----|----|----|----|----|
| 1             | 82 | 5  | 13 |    |    |
| 2             | 80 | 7  | 13 |    |    |
| 3             | 79 | 8  | 13 |    |    |
| 4             | 78 | 9  | 13 |    |    |
| 5             | 77 | 10 | 13 |    |    |
| 6             | 86 | 6  |    | 8  |    |
| 7             | 85 | 7  |    | 8  |    |
| 8             | 84 | 8  |    | 8  |    |
| 9             | 83 | 9  |    | 8  |    |
| 10            | 82 | 10 |    | 8  |    |
| 11            | 87 | 8  |    | 5  |    |
| 12            | 82 | 8  |    | 10 |    |
| 13            | 72 | 8  |    | 20 |    |

Hereinafter is reported on the experiments made with some of these alloys.

A ladle, coated with aluminous refractories, of 600 l. capacity was used in the experiments.

The temperature of the molten steel was in the range of 1590° C.—1630° C. The same steel and technique were used throughout.

#### Li-Al-Ca alloys

with pure Al, total inclusions p.p.m. 187, FeO 18%, Al<sub>2</sub>O<sub>3</sub> 31%, SiO<sub>2</sub> 30%, MnO 9%, others 12%

with alloy No. 6, total inclusions p.p.m. 160, FeO 14%, Al<sub>2</sub>O<sub>3</sub> 26%, SiO<sub>2</sub> 25%, MnO 17%, others 18%

with alloy No. 8, very strong agitation of the molten steel, total inclusions p.p.m. 191, FeO 17%, Al<sub>2</sub>O<sub>3</sub> 33%, SiO<sub>2</sub> 30%, MnO 10%, others 10%

with alloy No. 10 the operation resulted dangerous because too violent agitation of the molten steel occurred.

#### Li-Al-TR alloys

with alloy No. 1 total inclusions p.p.m. 146, FeO 11%, Al<sub>2</sub>O<sub>3</sub> 26%, SiO<sub>2</sub> 28%, MnO 15%, others 20%

with alloy No. 2 total inclusions p.p.m. 152, FeO 9%, Al<sub>2</sub>O<sub>3</sub> 30%, SiO<sub>2</sub> 28%, MnO 17%, others 16%

with alloy No. 5, same as alloy No. 10

The hereinafter listed alloys, from c onwards (not considering aluminum metal, named a, and alloy b, only used for comparative purposes), which are mentioned only as illustrative but not as limitative of the invention, have been successfully applied:

|            | Al    | Li  | TR                              | Ca | Ba | B   | Fe  |
|------------|-------|-----|---------------------------------|----|----|-----|-----|
| Reference: | 100.0 |     |                                 |    |    |     |     |
| a          | 90.0  | 0.5 | 10                              |    |    |     |     |
| b          | 99.5  | 3.5 | Preserved in a closed container |    |    |     |     |
| c          | 96.5  | 5.0 |                                 |    |    |     | 3.0 |
| d          | 86.2  | 0.8 | 13.0                            |    |    |     |     |
| e          | 92.5  | 1.5 | 6.0                             |    |    |     |     |
| f          | 91.9  | 3.6 | 4.5                             |    |    |     |     |
| g          | 84.6  | 5.4 | 10.0                            |    |    |     |     |
| h          | 90.0  | 1.4 | 8.0                             |    |    | 0.6 |     |
| i          | 94.0  | 1.0 | 5.0                             |    |    |     |     |
| j          | 88.0  | 2.0 | 10.0                            |    |    |     |     |
| k          | 91.7  | 0.8 |                                 |    |    | 7.5 |     |
| l          | 96.0  | 1.2 |                                 |    |    | 2.8 |     |
| m          | 96.3  | 2.5 |                                 |    |    | 1.2 |     |
| n          | 98.2  | 2.3 |                                 |    |    | 1.5 |     |
| o          | 96.0  | 1.0 |                                 |    |    | 3.0 |     |
| p          | 92.0  | 2.0 |                                 |    |    | 3.0 | 3.0 |
| q          | 96.8  | 1.2 |                                 |    |    | 2.0 |     |
| r          | 91.7  | 2.3 | 5.0                             |    |    | 1.0 |     |
| s          | 89.7  | 1.8 | 8.0                             |    |    | 0.5 |     |
| t          | 88.4  | 2.6 | 8.0                             |    |    | 1.0 |     |
| u          | 89.2  | 1.2 | 8.0                             |    |    | 1.6 |     |

Particularly good results have been obtained with the following standard alloys: s, m, n, d and l.

All the alloys of the present invention may be employed for the production of low, medium and high carbon steels, and also for the production of low, medium and high alloy steels as for example stainless steel, chrome and manganese steels.

The addition percentage of these alloys to the steel may vary depending on the steel-type treated and also on the employment field which the steel is destined to. In any

case these additions are limited as follows: from 0.01 to 0.16%, i.e. from 10 grs. to 1600 grs. per ton of liquid steel.

According to a preferred method the new alloys are added to the steel by plunging it down to the bottom of the filled ladle; alternatively the alloy may be introduced at the bottom of the ladle where thereafter the molten steel is poured.

Following these methods, the alloy uniformly reacts with all the liquid mass.

It is also possible to add the alloy in the furnace or in the ingot mold, in shapes such as stars, pellets, wires, etc.

The present invention may be successfully used in all those fields of metallurgical industry wherein Al has been used up to date to kill and refine steel, as well as to control its grain size to obtain higher purity qualities.

The invention is hereafter illustrated by the examples in which, for comparison purposes, the same steel are treated with Al alone and with alloys, consisting of or comprising Al-Li. All percentages are by weight.

The invention is hereafter illustrated by the following examples in which for comparison purposes the same steel was treated: with aluminum alone, Al 90%+TR 10%, and with Type A and C alloys of the invention. All percentages are by weight.

#### Example 1

The following steels:

Type "I": C 0.24—Mn 0.72—Si 0.26—P 0.02—S 0.03

Type "II": C 0.32—Mn 1.60—Si 0.25—P 0.02—S 0.03

Type "III": C 0.42—Mn 0.75—Si 0.25—P 0.015—S 0.03

treated in the molten state as indicated, thereafter normalized at 850° C. and tempered at 530° C., gave the following results

| Treated with—  | Alloy number | Tension strength, kg./mm. <sup>2</sup> | Yield strength, kg./mm. <sup>2</sup> | Elongation, percent | Reduction of area, percent | Resilience Charpy, kg./m./cm. <sup>2</sup> |
|----------------|--------------|----------------------------------------|--------------------------------------|---------------------|----------------------------|--------------------------------------------|
| Type I steel   |              |                                        |                                      |                     |                            |                                            |
| Al             | a            | 53.20                                  | 30.70                                | 30.00               | 51.20                      | 4.95                                       |
| Al-TR          | b            | 53.25                                  | 30.80                                | 30.60               | 53.40                      | 5.80                                       |
| Al-Li-TR       | n            | 53.25                                  | 31.40                                | 31.40               | 56.30                      | 6.74                                       |
| Type II steel  |              |                                        |                                      |                     |                            |                                            |
| Al             | a            | 65.20                                  | 44.50                                | 27.2                | 55.00                      | 6.32                                       |
| Al-TR          | b            | 65.60                                  | 44.60                                | 27.8                | 56.70                      | 6.48                                       |
| Al-Li-TR       | n            | 66.20                                  | 44.95                                | 28.6                | 60.50                      | 7.30                                       |
| Type III steel |              |                                        |                                      |                     |                            |                                            |
| Al             | a            | 65.6                                   | 39.10                                | 24.2                | 37.5                       | 2.54                                       |
| Al-TR          | b            | 65.7                                   | 40.20                                | 25.1                | 39.4                       | 2.81                                       |
| Al-Li-TR       | n            | 66.3                                   | 41.60                                | 27.8                | 45.6                       | 3.42                                       |

Analysis of the steels as above treated, made according to ASTM 45/63 test method gave the following type of inclusions:

| Alloy number   | A | B   | C     | D     | E   |
|----------------|---|-----|-------|-------|-----|
| Type I steel   |   |     |       |       |     |
| Treated with—  |   |     |       |       |     |
| Al             |   | 3/4 | 3     | 2 2/3 | 2   |
| Al-TR          | a | 4/5 | 2 2/3 | 1     | 2   |
| Al-Li-TR       | b | 3   | 1     | 1/2   | 0   |
|                |   |     |       |       | 1/2 |
| Type II steel  |   |     |       |       |     |
| Al             | a | 3/4 | 3     | 2     | 3   |
| Al-TR          | b | 3/4 | 3     | 2     | 3   |
| Al-Li-TR       | n | 2   | 0     | 0     | 1   |
| Type III steel |   |     |       |       |     |
| Al             | a | 3/4 | 3     | 2     | 2   |
| Al-TR          | b | 4/5 | 2 2/3 | 2     | 4   |
| Al-Li-TR       | b | 2   | 1/2   | 0     | 1   |
|                |   |     |       |       | 1/2 |

#### Example 2

A 12/14 manganese steel was treated in the molten state as follows, then austenized at 1100° C. and mill hammer casted therewith.

Analysis according to ASTM 45/63 gave the following types of inclusions:

|                 | Alloy number | A | B | C | D | E |
|-----------------|--------------|---|---|---|---|---|
| 5 Treated with— |              |   |   |   |   |   |
| Al              | a            |   |   | 1 | 2 | 1 |
| Al-TR           | b            |   |   | 1 | 3 | 2 |
| Al-Li-TR        | n            | 0 | 0 | 0 | 0 | 0 |

The results of the treatment are hereafter tabulated:

|                  | Alloy number | Mill hammers' hours of operation |
|------------------|--------------|----------------------------------|
| 10 Treated with— |              |                                  |
| Al               | a            | 22                               |
| Al-TR            | b            | 43                               |
| Al-Li-TR         | n            | 71                               |

#### Example 3

20 AISI/1040 steel of the following composition: C 0.43; Mn 0.72; Si 0.28; S 0.02; P 0.016 was treated in the molten state as follows: thereafter normalized at 850° C. and tempered at 530° C. The following results were obtained:

|                  | Alloy number | Tension strength | Elongation, percent | Reduction of area | Resilience (Charpy, kg./cm. <sup>2</sup> ) |
|------------------|--------------|------------------|---------------------|-------------------|--------------------------------------------|
| 25 Treated with— |              |                  |                     |                   |                                            |
| Al               | a            | 89.0             | 16.2                | 38.3              | 2.7                                        |
| Al-Li-Ca         | s            | 88.7             | 19.3                | 47.1              | 3.8                                        |

|                  | Alloy number | A     | B   | C | D | E |
|------------------|--------------|-------|-----|---|---|---|
| 30 Treated with— |              |       |     |   |   |   |
| Al               | a            | 4-3-2 | 3-2 | 2 | 1 | 1 |
| Al-Li-Ca         | s            | 0-1   | 0   | 0 | 1 | 0 |

Only from an interpretative point of view, which is in no way limitative upon the above disclosed invention, it 55 may be thought that the highly advantageous results obtained with the peculiar Al-Li alloys of the present invention derive from an action both chemical and physical of Li. As a matter of fact it seems that this metal has a high reaction rate towards the oxygen present in the steel so forming the low-density-lithium oxide which further reacts with  $Al_2O_3$  and with the other oxides of refractory character present in the steel leading to low-melting complex products which easily coagulate and decent gathering in the slag.

Moreover Li when coming into contact with molten steel, evaporates, thus exerting a strong action on the bath i.e. of bubbling and dragging the impurities into the slag.

60 Of course, the exploitation of these so advantageous characteristics of Li is rendered possibly by the fact that I use it only in critically limited amounts, diluted into the active Al, and also by the fact that I have found the manner to stabilize the Al-Li alloys containing from 1.2 to 75 8% of Li.

It has been impossible up to now to fully understand the stabilizing action exerted on the Al-Li alloys by the elements Fe, Ba, Ca, TR.

However such a circumstance is of no consequence for the purposes of the invention.

What is claimed is:

1. In the method of deoxidizing, depurating, killing and refining steels by adding aluminum alloys to the molten steel, the improvement consisting of using as said aluminum alloy an alloy consisting of more than 98.8% to 99.7% aluminum and 0.3% to less than 1.2% lithium in an amount of 0.01-0.16% based on the weight of the steel.

References Cited

UNITED STATES PATENTS

|           |         |                 |         |
|-----------|---------|-----------------|---------|
| 2,233,726 | 3/1941  | Belding         | 75-58   |
| 2,360,717 | 10/1944 | Phelps          | 75-58 X |
| 2,609,289 | 9/1952  | McKinney et al. | 75-58 X |
| 2,683,661 | 7/1954  | Tisdale et al.  | 75-58 X |
| 2,705,196 | 3/1955  | Wever et al.    | 75-58   |

15 14,693  
10 3,414,042  
20 3,623,862  
75-58

|           |         |                    |         |
|-----------|---------|--------------------|---------|
| 2,705,673 | 8/1955  | Jordan             | 75-58 X |
| 2,808,327 | 10/1957 | Pierce             | 75-58   |
| 2,836,489 | 5/1958  | Henke              | 75-58   |
| 2,873,188 | 2/1959  | Bienosek           | 75-58 X |
| 2,980,529 | 4/1961  | Knapp et al.       | 75-58 X |
| 3,058,822 | 10/1962 | Volianik           | 75-58 X |
| 3,290,142 | 12/1966 | Loomis             | 75-58   |
| 3,314,782 | 4/1967  | Arnaud             | 75-58 X |
| 3,383,202 | 5/1968  | Lynch              | 75-58 X |
| 3,414,042 | 12/1968 | Behrens et al.     | 75-58 X |
| 3,623,862 | 11/1971 | Spengler et al.    | 75-58 X |
| 1,620,081 | 3/1927  | Czochralski et al. | 75-138  |

FOREIGN PATENTS

1902 Great Britain.

L. DEWAYNE RUTLEDGE, Primary Examiner

P. D. ROSENBERG, Assistant Examiner

U.S. CL. X.R.